

## UNITED STATES PATENT OFFICE

2,507,183

## SILVER BLEACH FOR COLOR MATERIALS

Lot S. Wilder, Rochester, N. Y., and Kent C. Brannock, Oak Ridge, Tenn., assignors to Eastman Kodak Company, Rochester, N. Y., a corporation of New Jersey

No Drawing. Application March 23, 1945,  
Serial No. 584,494

1 Claim. (Cl. 95—88)

1

This application relates to color photography and particularly to the removal of silver images from emulsion layers in color photography.

In photographic color processes in which a colored image is formed by development with a primary aromatic amino developing agent in the presence of a coupler compound, the silver images formed during development are present in the emulsion layer together with dye images. These silver images are generally removed by converting them to a silver salt which is soluble or which is removed by hypo. A bath of this type containing potassium ferricyanide and potassium bromide is disclosed in Mannes, Godowsky and Wilder U. S. Patent 2,252,718, granted August 19, 1941.

Silver bleach baths containing quinone and an acid have also been used for removal of silver. A bath of this type is disclosed in Mannes and Godowsky U. S. Patent 2,113,329, granted April 5, 1938. These quinone bleach baths cannot be used in the final stages because they destroy the image dyes as well as convert the silver to a silver salt. A quinone bleach bath suitable for removal of silver in the presence of a dye image is described in Vittum U. S. patent application Serial No. 541,843, filed June 23, 1944, now abandoned.

Quinone bleach baths are inconvenient to prepare because the quinone dissolves very slowly in aqueous solutions. The common organic solvents are inconvenient or adversely influence the solution. Quinone is quickly soluble in hot glacial acetic acid, but this requires handling hot liquid and is an inconvenience in the preparation of the bleach bath. Any liquid is undesirable where the ingredients of the bath must be packaged for sale and kept for a period of time before being purchased by the ultimate user.

It is, therefore, the principal object of the present invention to provide a simple and convenient method for the preparation of quinone bleach baths for use in color photography. A further object is to provide a bleach bath which may be packaged and kept in dry form. Other objects will appear from the following description of our invention.

These objects are accomplished by using as the source of the quinone a mixture of hydroquinone and an oxidizing agent for the hydroquinone which converts it to quinone in acid solution. Suitable oxidizing agents for this purpose are alkali metal salts of oxygen acids capable of oxidizing hydroquinone to quinone. Suitable alkali metal salts are the sodium, potassium, and ammonium salts, such as ammonium persulfate, potassium permanganate and potassium dichromate.

In the preparation of bleach baths according to our invention, the hydroquinone is mixed with

2

the oxidizing salt in aqueous acid solution. The solution may contain glacial acetic acid as in the case of the prior art quinone bleach baths, although this is unnecessary. Acids which may be used include hydrochloric and sulfuric acid, or the acid may be obtained in solution from sodium acid sulfate or sulfamic acid. The bleach bath also may contain a soluble bromide or chloride to cause the formation of silver halide from the oxidized silver.

When packaged in dry form, the bleach baths of our invention preferably contain the hydroquinone in one compartment and the oxidizing agent and potassium bromide in another compartment. If a dry acid former, such as sodium acid sulfate, is used, it may be placed in the container with the hydroquinone. By "acid former" we mean a substance which forms an acid when dissolved in water, such as sodium acid sulfate, sulfamic acid, etc.

The following formulas illustrate bleach baths prepared according to our invention.

## Formula 1

|    |                           |       |    |      |
|----|---------------------------|-------|----|------|
| 25 | Hydroquinone              | ----- | g  | 2.5  |
|    | Ammonium persulfate       | ----- | g  | 5.14 |
|    | Potassium bromide         | ----- | g  | 10   |
|    | Glacial acetic acid       | ----- | cc | 5    |
|    | Hydrochloric acid (conc.) | ----- | cc | 5    |

30 Water to 1 liter.

## Formula 2

|                           |       |    |     |
|---------------------------|-------|----|-----|
| Hydroquinone              | ----- | g  | 2.5 |
| Potassium permanganate    | ----- | g  | 1.4 |
| 35 Potassium bromide      | ----- | g  | 10  |
| Sulfuric acid (conc.)     | ----- | cc | 1   |
| Glacial acetic acid       | ----- | cc | 5   |
| Hydrochloric acid (conc.) | ----- | cc | 5   |

Water to 1 liter.

## Formula 3

|                              |       |    |     |
|------------------------------|-------|----|-----|
| Hydroquinone                 | ----- | g  | 2.5 |
| Potassium dichromate         | ----- | g  | 2.2 |
| Potassium bromide            | ----- | g  | 10  |
| Sulfuric acid (conc.)        | ----- | cc | 1   |
| 45 Hydrochloric acid (conc.) | ----- | cc | 5   |

Water to 1 liter.

The following formula illustrates a dry powder mixture for preparing one liter of solution according to our invention:

## Formula 4

|          |       |   |    |  |
|----------|-------|---|----|--|
| A        |       |   |    |  |
| 55 NaHSO | ----- | g | 28 |  |

|                      |       |   |      |  |
|----------------------|-------|---|------|--|
| Hydroquinone         | ----- | g | 1.25 |  |
| B                    |       |   |      |  |
| Potassium dichromate | ----- | g | 1.5  |  |

|                   |       |   |    |
|-------------------|-------|---|----|
| Potassium bromide | ----- | g | 10 |
|-------------------|-------|---|----|

## Formula 5

|                      |         |
|----------------------|---------|
| Sulfamic acid        | g. 12   |
| Hydroquinone         | g. 1.25 |
| Potassium dichromate | g. 1.5  |
| Potassium bromide    | g. 10   |
| Water to 1 liter.    |         |

In place of quinone, derivatives of quinone, such as chloroquinone or toluquinone may be used. The bleach bath in use is followed by a dilute solution of sodium bisulfite, for example, a 1% solution of bisulfite to react with the retained quinone, and the photographic element is then fixed for about 4 minutes in hypo, washed and dried.

It will be understood that the examples and formulas included herein are illustrative only and that our invention is to be taken as limited only by the scope of the appended claim.

## We claim:

A dry powder composition for preparation of an acid quinone bleach bath by mixing with water, comprising hydroquinone, sodium hydrogen sulfate, and potassium dichromate.

LOT S. WILDER.  
KENT C. BRANNOCK. 25

## REFERENCES CITED

The following references are of record in the file of this patent:

## UNITED STATES PATENTS

| Number    | Name           | Date          |
|-----------|----------------|---------------|
| 1,755,129 | Pomeroy        | Apr. 15, 1930 |
| 1,755,130 | Pomeroy        | Apr. 15, 1930 |
| 1,966,330 | Burwell        | July 10, 1934 |
| 1,969,479 | Seymour        | Aug. 7, 1934  |
| 2,019,718 | Mannes et al.  | Nov. 5, 1935  |
| 2,059,887 | Mannes et al.  | Nov. 3, 1936  |
| 2,113,329 | Mannes et al.  | Apr. 5, 1938  |
| 2,158,186 | Hickman et al. | May 16, 1939  |
| 2,195,419 | McQueen        | Apr. 2, 1940  |
| 2,313,523 | Donovan et al. | Mar. 9, 1943  |

## OTHER REFERENCES

Conant, "The Chemistry of Organic Compounds," The Macmillan Co., New York, 1936; page 414 cited.

Wall, "Photographic Facts and Formulas," American Photographic Publishing Company, 1924; page 240 cited.